

## UNITED STATES PATENT OFFICE

MARCUS A. GROSSMANN, OF CANTON, AND DAVID WILLIAMS, OF MASSILLON, OHIO,  
ASSIGNORS TO CENTRAL ALLOY STEEL CORPORATION, OF MASSILLON, OHIO, A COR-  
PORATION OF NEW YORK

## STEEL

No Drawing.

Application filed July 28, 1927. Serial No. 209,169.

The present invention has for its object a new and improved steel which shall be less subject to corrosion than steel as now made.

5 We believe that the corrosion of steel is promoted in part at least by the presence in it of dissolved nitrogen and iron nitrides as well as by the presence of dissolved oxygen. This conclusion is based in part on

10 certain work which has recently been done in connection with oxygen determination by the use of the apparatus developed by the Bureau of Standards of the United States.

15 The present invention has to do with the conversion of the dissolved nitrogen and iron nitrides into a crystalline form by which corrosion is not promoted. The element zirconium has the peculiar quality of uniting with dissolved nitrogen and iron nitrides

20 to form zirconium nitride crystals and when this occurs in molten steel the zirconium nitride crystals are largely carried to the top of the ingot and form a slag or to some extent remain included in the steel, but when

25 so included being inert do not appear to promote corrosion at any rate in an active manner. Accordingly our present invention consists in its broadest aspect in the use of zirconium to convert the dissolved nitrogen

30 and iron nitrides in molten steel, more particularly effervescent steel, into zirconium nitride crystals. We find in practice however that the ordinary commercial forms of zirconium contain elements which interfere

35 with the effectiveness of the zirconium or produces other detrimental results on the product so that the mere application of ferro-zirconium to molten effervescent steel does not appear to be practical. Ferro-zirconium as ordinarily produced contains silicon, the effect of which on the steel is to cause the effervescent steel to rise in the mold so that the ingot is porous and less dense.

40 We have found however that the application of ferro-zirconium in the presence of a fluorine compound such as fluorspar (calcium fluoride) or in fact any of the fluorine compounds except aluminum fluoride tend to cause the effervescent steel to fall in the mold and thus to counteract the ill effects of the

silicon in the ferro-zirconium. In fact if proper proportions of the fluorine compound are employed an effervescent steel of exceptional density can be produced. The fluorine compound does not interfere with the 55 action of the zirconium on the dissolved nitrogen and iron nitrides and the result is that we are able to obtain a steel (particularly an effervescent steel) in which dissolved nitrogen and iron nitrides have been converted 60 into inert zirconium nitride crystals which are either carried off in the slag or remain to a small extent in the metal and that the ingot so produced is exceptionally free 65 from porosity and has a high density.

While we have not yet determined the limits within which the amount of zirconium and fluorine may be varied and still be effective for the purpose intended, we have found that the following proportions give 70 good results. Molten steel 3000 pounds to which is added 4 ounces of commercial 35% ferro-zirconium and 8 ounces of calcium fluoride or fluorspar which are added in the mold after a small amount of the molten 75 steel has been poured into the mold and before it has been filled. While we prefer to add the zirconium and fluorine compounds in the mold it is obvious that it can be added at other times in process of manufacture, for example, in the ladle.

We also believe and know of no reason to doubt that our invention is applicable not only to pure steels by which we mean steels containing no alloying metal, but also to 85 some at least of the alloy steels containing alloying metals, particularly copper, molybdenum and nickel.

What we claim is:—

1. The method of improving the quality 90 of an effervescent steel which comprises adding a fluorine compound and ferro-zirconium containing silicon.

2. The method of improving the quality 95 of an effervescent steel which comprises converting the dissolved nitrogen and iron nitrides by the action of ferro-zirconium containing silicon in the presence of a fluorine compound.

3. The method of improving the quality 100